

## UNITED STATES PATENT OFFICE

JAMES B. GRENALE, OF BALTIMORE, MARYLAND, ASSIGNOR OF ONE-HALF TO WILLIAM W. VARNEY, OF BALTIMORE, MARYLAND

## PROCESS OF MAKING AN ALLOY

No Drawing.

Application filed October 21, 1929. Serial No. 401,374.

The object of my invention is the production of an alloying element which may be used either by itself in commercial production, or alloyed with other metals.

5 A further object of my invention is the production of an alloy that will withstand the corrosive effect of the surroundings in which it may be used and at the same time maintain the cutting edge of implements containing the same.

10 A further object of my invention is the producing of an alloy which is superior to high speed steels now commonly used in making cutting tools, which in addition to having the required hardness necessary to perform the functions in cutting operations, is extremely tough and has a very high melting point.

15 A further object of my invention is the production of an alloy of the character and characteristics set forth herein which is capable of being forged, hammered, or otherwise worked into various forms, and which is particularly adapted for use in the manufacture 20 of knife blades, and surgical and dental instruments.

25 A further object of my invention is the providing of an alloy having the characteristics herein enumerated, and which is not attacked by cutting compounds, caustics and acids usually employed in the cutting of hard metals, such as nickel-chrome, vanadium steels and manganese steels.

30 A further object of my invention is the production of an alloy, as herein suggested, which possesses a high and permanent lustre such as is required or desirable in metals for knife blades, surgical and dental implements.

35 A further object of my invention is the production of an alloy as suggested herein, which is substantially free from injurious impurities, especially such impurities as carbon, silicon, sulphur and like materials which seriously interfere with the non-tarnishing properties of alloys.

40 With the foregoing and other objects in view, my invention consists of the methods employed, combination and arrangement of 45 systems and means as hereinafter specifically

provided, but it is understood that changes, variations and modifications may be resorted to which come within the scope of the claim as hereunto appended.

I have discovered that an alloy of uranium, 55 zirconium and manganese, in proper proportions, has all the desired properties set forth herein. The percentages of uranium, zirconium and manganese may be varied within a considerable range. I have found that an 60 alloy containing about 70% of uranium, 25% zirconium and 5% of manganese is particularly adapted for use in making high speed tools, knife blades, dental and surgical instruments, and the like.

65 I will describe one method of producing the alloy mentioned herein—

I reduce ores containing oxides of uranium, 70 zirconium and natural oxide of manganese in an electric furnace in a reducing atmosphere such as is present when a carbon crucible, or carbon electrodes, are employed. I have discovered that the mixture of oxides of 75 uranium and zirconium melt at lower temperatures than either of the pure metals, so that the process of melting the oxides is more economical and can be more easily accomplished than melting the pure metals themselves.

80 The oxides are introduced into an electric furnace, rammed in and closely packed and covered with pure carbon, such as lamp black, charcoal, etc., and subjected to a high temperature, preferably, from about 2500 to 2600 degrees C. until a freely fluid alloy of uranium and zirconium is obtained. The 85 temperature is then slightly lowered to about 2300 to 2400 degrees C., when the manganese in the state of a natural oxide is added.

85 The alloy, after it has become freely fluid, is maintained at a temperature sufficiently high to keep it freely fluid for a substantial period of time, preferably about 15 minutes. The temperature is then reduced until the alloy is in a less fluid condition, and this temperature is maintained for a considerable period, preferably for about 15 minutes to eliminate the sonums. Caution: If the alloy is kept in a freely fluid condition at a high temperature for too long a time, it will have

a crystalline structure when cool, and the product made therefrom will be somewhat brittle instead of having a high degree of toughness. The purpose, therefore, of reducing the temperature of the alloy after it has become freely fluid, and holding it at this reduced temperature, is to prevent crystallization of the alloy upon cooling, and to produce an alloy of extreme toughness.

10 After the alloy has been maintained at a reduced temperature for a substantial period of time, it is poured directly into suitable molds with proper neutral lining, and the articles made are ground into the required shapes and condition for use.

The above alloy, when poured into molds having a proper lining of a neutral, highly refractory substance, will give a superior product which is free from checks and blow-holes, provided the flask and lining are heated prior to pouring. I heat the mold to 1200 degrees F. The alloy above described may contain some iron, up to possibly 2%, without the least detriment to the products produced. The alloy, after being cast in the mold, requires no further heat treatment or tempering before grinding into the shapes required.

I have found that this alloy may be advantageously added to or alloyed with iron, and that the resulting alloy has certain superior qualities over high speed steels. The proportion of iron which may be alloyed with my alloy may range from 2% to 95%; as the amount of iron which is added is increased, the alloy becomes softer. If an amount of iron between 2% and 10% be added to my alloy, the resulting product need only be cast into molds and ground into the shape required. If, however, the amount of iron which is added to my alloy is greater than 10%, say, between 10% and 95%, the resulting product is so soft that after being poured into a mold it must be heat treated, or tempered, in a manner similar to the heat treatment of high speed steels before it will be sufficiently hard to be used as a high speed cutting tool.

I have found that my alloy, when containing 10% or more of iron, may be readily forged between the critical range of temperatures of 1400 and 1800 degrees F.

One method of obtaining uranium oxide which I have used with satisfactory results, is as follows:

The ore is roasted with an alkali until thoroughly fused then washed with hot water until free of iron, and dissolved with  $HNO_3$ . Evaporate the  $HNO_3$  solution obtained to a volume of about 40% and cool. After making neutral with  $NH_4OH$ , add about 5% of  $HC_2H_3O_2$  and 15% of  $HPO_4$ , and heat the mixture to boiling, when a white precipitate of uranium is formed. Cool to coagulate the precipitate, and wash and ignite to  $U_3O_8$ .

When uranium and zirconium are melted together they tend to separate into two layers due to their different specific gravities and to the low solubility of either metal with reference to the other when mixed together. Even in the liquid condition uranium and zirconium do not mix completely, but form two layers, one rich in uranium and the other rich in zirconium. When allowed to rest quietly at very high temperatures these two layers approach each other in composition; in other words, the solubility of each metal in the other increases with increased temperature; on the other hand, the solubility decreases with decreased temperature.

When uranium and zirconium are melted and stirred in the presence of manganese a fine dissemination of the two metals is brought about and maintained in the cooled alloy. The metals do not actually dissolve in each other, but the dispersion is so fine that the unaided eye is unable to distinguish the separate metals. The microscope reveals the uranium constituent as a continuous phase completely surrounding the fine globules or separated particles of zirconium. Examination with a micrometer microscope of the zirconium particles will show very fine minute crystal structure. The action of manganese causes the uranium to solidify first as a dentritic skeleton rejecting practically all of the zirconium, the dentritic skeleton finally becoming continuous and completely surrounding the disconnected particles of zirconium. After the uranium is frozen and the alloy continues to cool, the dentritic skeleton completely surrounds the zirconium binding the metals together in what appears to be a solid alloy by means of a continuous net work.

The separated crystals of zirconium cannot be lignited away from the alloy, for they are enclosed in the continuous skeleton of uranium which requires a high temperature to melt.

One method of obtaining zirconium oxide, which I have used with satisfactory results, is as follows:

Brazilian ore is thoroughly crushed, ground and pulverized (150-200 mesh) and added to a molten bath of equal parts of sodium chloride, sodium carbonate and sodium bisulphate. A temperature high enough to volatilize the alkalis must be reached, which may be determined by the amount of carbon dioxide liberated, and maintained at a dark red heat until all of the carbon dioxide is expelled. The major portion of the iron, practically all of the silica, and all of the accompanying rare earths having high solution pressure either go into solution and are recovered from the mother liquor, or, as in the case of silica, are completely vaporized and are driven off with the carbon dioxide.

The resultant fused mass, after cooling is thoroughly leached with water, leaving a

crystalline sodium zirconate which is decomposed by hydrochloric acid. All of the books and other writings which the applicant has examined, state that sodium zirconate is soluble in water; this the applicant finds to be a grave error, as he has found that sodium zirconate is insoluble in water, as a matter of fact, the insolubility of the residue in water is sufficient proof that only zirconia is present.

10 ent.

Further purification:

The zirconate is then dissolved in hydrochloric acid (dilute) and evaporated to dryness, this being repeated to separate any silica 15 and to drive off such hydrochloric acid as remained. The dried mass is leached with dilute HCl and zirconia precipitated as hydroxide with ammonia. This hydroxide is dissolved in hot concentrated HCl, to a solution 20 evaporated to dryness and the crude zirconyl chloride washed with water, thus removing most of the iron present. The zirconyl chloride is then repeatedly crystallized from boiling HCl. This chloride still 25 contains some silica which may be removed by dissolving in water and filtering; several crystallizations from water giving a very pure chloride. For the complete removal of all impurities it is necessary to transform this 30 oxychloride into tetrachloride and sublime it repeatedly. On the ignition the chloride yields the oxide containing traces of chlorine. For the pure oxide it is necessary to precipitate the hydroxide, wash and ignite.

35 I use natural manganese oxide, in the mixture above described.

I have discovered that not more than 95% of iron can be added to my alloy, as any greater percentage of iron will form impurities of iron oxide which upon slagging off 40 will cause the zirconium metal to burn to its oxide with a resultant ferric-zirconic oxide, resulting in a complete loss of alloy.

In these specifications and claims, when I 45 use the term, "alloy," I mean an allotropic mixture wherein the metals undergo a physical change and not necessarily a chemical change.

Having thus described my invention, what 50 I claim and desire to secure by Letters Patent is:

The process of producing a dentritic alloy containing uranium, zirconium and manganese consisting of co-mingling oxides of zirconium and uranium, smelting the same in contact with carbon whereby a fluid melt of 55 said two elements intimately associated is produced, then lowering the temperature of the said molten mass, and then adding the manganese oxide for the purpose of diffusing the uranium to form the dentritic structure.

JAMES B. GRENAGLE.